

Patented Oct. 27, 1925.

## UNITED STATES PATENT OFFICE.

CARL D. HOCKER, OF EAST ORANGE, NEW JERSEY, ASSIGNOR TO WESTERN ELECTRIC COMPANY, INCORPORATED, OF NEW YORK, N. Y., A CORPORATION OF NEW YORK.

## SOLVENT AND VEHICLE FOR RESINOUS AND GELATINIZED MATERIAL.

No Drawing.

Application filed December 11, 1919. Serial No. 344,178.

*To all whom it may concern:*

Be it known that I, CARL D. HOCKER, a citizen of the United States, residing at East Orange, in the county of Essex, State of New Jersey, have invented certain new and useful Improvements in Solvents and Vehicles for Resinous and Gelatinized Material, of which the following is a full, clear, concise, and exact description.

10 This invention relates to vehicles for resinous and similar substances used in varnishes, enamels, impregnating compounds, japans, lacquers, and the like.

Natural resins such as used for bases of the so-called varnish gums and spirit lacquers, vary greatly in their solubility. Some are soluble in common solvents such as alcohol, benzol, carbon-bisulphide, turpentine, petroleum products and others can be brought into solution only by special solvents or mixtures unless given some preliminary treatment, such as fusion. Drying oils also have been used to some extent as vehicles for such natural resins. If the varnish gums which are employed are those which require a preliminary treatment, the fusion operation necessary to render them soluble involves a considerable loss of material. This is of course undesirable.

30 Take for example the usual method employed in treating gums for use in making varnishes. The resin must be subjected to a preliminary fusion until all the residue can be completely incorporated with the oily vehicle or solvent. A considerable amount of the raw material, depending upon the hardness of the resin, is thus lost. If the resin be treated with drying or semidrying oils, only a limited amount of the resin may be dissolved, the resulting mixture being comparatively low in resin content.

It is well known that if vegetable oils are subjected to a heat treatment under the proper conditions of pressure, i. e., either atmospheric or diminished pressure depending on the nature of the oil, a gelatinous product may be obtained. In case of those vegetable oils which will gelatinize on heating, the oil will only dissolve about an equal weight of the gel, and for this reason the resulting solutions have been relatively dilute.

An object of the invention is to produce a vehicle in which these resinous or gelatinized materials may be incorporated, i. e., resins,

the gelatinized products of vegetable oils and the gelatinous masses formed by the overheating of an oil and resin.

By completely saponifying drying oils such as linseed and Chinese wood oils, or 60 semi-drying oils such as corn, cotton-seed, sesame, rapeseed, and castor oils, there is produced a polyacid alcohol, glycerine, on the one hand and, on the other, alkali salts from which can be precipitated two or more free fatty acids. The following fatty acids have been found as being derived in this manner from the oils above mentioned; oleic, stearic, palmitic, 65 myristic, linolenic, isolinolenic, elaeomargaric, arachidic, erucic, eramic, ricinoleic, and dihydroxystearic. The free fatty acids may be derived from the vegetable oils by saponifying the oils with an excess of a solution of caustic soda or potash in water, and after 70 complete saponification, decomposing the resulting soaps with a dilute acid, such as hydrochloric acid or sulphuric acid, washing and filtering. One laboratory process which has been used to accomplish this is the following: One kilo of the oil is heated to about 80° C. and a solution of 50 grams caustic soda in 600 c. c. of water is added with constant stirring. The emulsion formed is heated to boiling, and a solution of 150 grams 75 caustic soda in 1200 c. c. water is added. The mass is kept boiling until complete saponification has taken place, and then 3 liters of water are gradually added until a clear solution has been obtained. The fatty acids are set free by adding a dilute solution of sulphuric acid (10%) with brisk stirring to the soap solution until the watery underlying layer, which contains the glycerine, shows a distinct acid reaction to litmus paper, and fatty acids, which have been set free, form a uniform clear layer on top of the water. The water is drawn off, and the fatty acids washed free from mineral acids 80 and salts by repeated treatment with hot water, after which they are filtered and dried. By taking one of the above fatty acids or a mixture of them as is obtained from a vegetable oil by the above process, and adding to it either a resin, the gelatinized product formed by the heating of a 85 vegetable oil at atmospheric or diminished pressure, the gelatinized product formed by the combination of a resin with a vegetable oil, or the gelatinized product formed by the 90

100 vegetable oil at atmospheric or diminished pressure, the gelatinized product formed by the combination of a resin with a vegetable oil, or the gelatinized product formed by the 105

action of glycerine on a resin, it has been found that a homogeneous body is readily obtained. In the case of the treatment with the acids of the gelatinized product formed by the heating of the vegetable oil at atmospheric or diminished pressure, the homogeneous body obtained will be a liquid, while in the cases of resins or their gelatinized products, the character of this compound will depend upon the proportion of the acids employed, and the nature of the solid resinous or gelatinized material used.

The adaptation of such compounds as mentioned herein for enamels, impregnating compounds, japans, lacquers, and varnishes has been proven by tests which have been made and the value of the discovery of this property of the free fatty acids and its application will be apparent to one skilled in the art.

An example of the use of these free fatty acids as vehicles for the above mentioned substances is shown in the preparation of a liquid composition for application to electrical conductors as an insulating enamel or japan. A basic material for this composition is formed, preferably, from Congo copal and Chinese wood oil. By saponification of the Chinese wood oil and subsequent separation from the glycerine and precipitation of their alkali salts by process described above, a mixture of fatty acids consisting largely of oleic and elaeomargaric acids is obtained. Three parts of the Congo copal are added to two parts of this mixture of free fatty acids and heat is applied until a temperature of from 250 to 300 degrees centigrade is reached. After maintaining the mixture at this temperature for two hours, it is allowed to cool. The result is a wax-like product which may readily be used as a basic material in making compounds for the enameling of wire.

In the manner described above, after subjecting a vegetable oil, such as Chinese wood oil to heat and obtaining a gelatinized product therefrom, the free fatty acid may be added thereto; and the whole heated to a homogeneous state, thereby yielding a satisfactory material for liquid coating compositions. So also the product formed by the heating of a vegetable oil with a resin may be dissolved readily in either one or more of the free fatty acids, giving a uniform, syrupy composition.

Moreover, as will be seen from my prior Patent No. 1,422,861, granted July 18, 1922, the free fatty acids afford a means by which resins may be more easily treated with glycerine in order to form the specific coating composition covered by that application.

While there has been named herein a specific number of resinous materials which

may be utilized in preparing liquid coating compositions according to the invention, it is intended to include all substances of resinous or gelatinized-oleaginous nature, which are adapted for such use when one or more of the free fatty acids are used as the vehicle.

In order that it may be understood what acids are intended to be included as belonging to the fatty acid class, a word of explanation is considered to be necessary. Various textbooks which contain matter relating to the chemical composition of such substances differ in their classification of the fatty acids. As used in this specification, the term "fatty-acids" is considered to include any and all classes embraced by the following outline:

1. Acids of the acetic series,  $C_nH_{2n}O_2$ .
2. Acids of the oleic series,  $C_nH_{2n-2}O_2$ .
3. Acids of the series  $C_nH_{2n-4}O_2$ , which includes the open chain and cyclic series.
4. Acids of the linoleic series,  $C_nH_{2n-6}O_2$ .
5. Acids of the clupanodonic and the  $C_nH_{2n-8}O_2$  series.
6. Hydroxylated or carboxylated acids of any of the above series.

What is claimed is:

1. The process of forming a composition of matter which comprises adding free fatty acid to gelatinized castor oil.
2. The process of forming a composition of matter which comprises gelatinizing vegetable oil and resin, and adding free fatty acid thereto.
3. The process of forming a composition of matter which comprises gelatinizing castor oil and copal, and adding free fatty acid thereto.
4. A composition of matter comprising gelatinized castor oil and free fatty acid.
5. A composition of matter comprising free fatty acid, and gelatinized castor oil and copal.
6. The process of forming a composition of matter which comprises adding free fatty acid to gelatinized castor oil, and heating these ingredients to form a homogeneous mass.

7. The process of forming a composition of matter which comprises gelatinizing vegetable oil and resin, adding free fatty acid thereto and heating the resulting product to a homogeneous state.
8. The process of forming a composition of matter which comprises gelatinizing castor oil and copal, adding free fatty acid thereto and heating the resulting product to a homogeneous state.

In witness whereof, I hereunto subscribe my name this 10th day of December A. D., 1919.

CARL D. HOCKER.